

## UNITED STATES PATENT OFFICE

EDWIN J. BOHNEN, OF CHICAGO, ILLINOIS, ASSIGNOR TO STANDARD OIL COMPANY, OF WHITING, INDIANA, A CORPORATION OF INDIANA

## METHOD OF LUBRICATING HIGH TEMPERATURE EQUIPMENT FOR COOKING FOOD

No Drawing.

Application filed September 16, 1929. Serial No. 393,110.

This invention relates to a method of lubricating high temperature equipment for cooking food, an example of such equipment being a continuous baking oven.

5 Continuous baking ovens are designed for baking bread in passage through the oven, the bread being placed upon trays and the trays being carried through on a continuous chain belt. For lubricating the chain belt, it  
10 is important to employ a lubricant having good penetration, which will not form objectionable odors when exposed to the high temperatures of the oven and which will provide effective lubrication under these severe con-  
15 ditions.

I have found that a satisfactory lubricant can be produced by suspending graphite in a highly refined light oil. The graphite, when deposited upon the bearings, is able to with-  
20 stand the high temperatures of the baking oven and properly lubricates the moving parts of the belt. It is carried readily to all the bearing surfaces by the light oil in which it is suspended, and the light oil vaporizes before  
25 temperatures are reached in which it might be decomposed. The objectionable fumes and odors, which are formed by the decom-  
position of ordinary graphite greases and oils, when such high boiling oils are employed un-  
30 der conditions of high temperature, are thus avoided.

In practice, it has been found extremely difficult to keep the lubricant from coming in contact with the bread during the handling  
35 of the material, both before and after applica-  
tion to the chains. The highly treated light oil, which I employ to carry the graphite in suspension, is substantially odorless and does not contaminate the bread if brought in contact therewith. This oil is  
40 preferably made from straight run refined oil by treating with 93% sulfuric acid. Preferably, I employ an oil having a boiling point of about 350° F. and an end point of  
45 about 575° F., although oils having a lower boiling point and a higher end point have been satisfactorily used. For example, if desired, treated light oils, having an end point as high as 700° F., may be satisfactorily used. A refined oil of the type described is

found to have lost its characteristic kerosene or other hydrocarbon odor after having been treated with 8 pounds of acid per barrel of oil. If desired, the oil may be treated in suc-  
55 ccessive batches with varying amounts of acid per treatment. For example, it has been found satisfactory to make four successive treats with 2 pounds of acid per barrel in each treat. The finished oil is substantially odorless, most of the objectionable constitu-  
60 ents having been treated out by the acid.

In preparing the lubricant, graphite in a very finely divided form is employed; for example, graphite sufficiently finely ground to enable it to remain in suspension in the oil for five minutes or more. I have satisfactorily used a fine form of graphite, known commercially as number 205 graphite. This has been found to remain suspended in the light oil for about 10 minutes, while ordinary  
70 amorphous graphite, normally employed in graphite greases and oils, remained in sus-  
pension for only about 10 seconds.

In practice, it has been found that the highly treated light oil graphite lubricant  
75 serves to carry the graphite readily to the bearing surfaces of the chain belt, does not decompose to form objectionable odors or fumes, but vaporizes readily after having served its function of carrying graphite to  
80 the bearings, and even when brought in contact with the bread passing through the oven, does not contaminate it or render the bread product objectionable. The highly refined light oil has high wetting power, good penetra-  
85 tion, and is well adapted for carrying graphite in suspension.

Although the present invention has been described in connection with the details of a specific example thereof, it must be under-  
90 stood that it is not intended that such details shall be limitative of the scope of the invention, except insofar as included in the accom-  
panying claim.

I claim:

The method of lubricating high tempera-  
ture equipment for cooking food which com-  
prises applying thereto at low temperatures  
a suspension of graphite in a treated, taste-  
less, non-odorous, light hydrocarbon oil  
100

whereby the oil penetrates and carries the graphite into remote portions of said equipment, and vaporizing said oil in situ, leaving the graphite in said remote parts of the equipment to serve as a lubricant, the vaporized oil being unobjectionable because it is tasteless and non-odorous.

EDWIN J. BOHNEN.

10

15

20

30

40

45

50

55

65